

Dec. 11, 1956

J. H. FUQUA ET AL

2,773,761

FERROUS CHROME ALLOY

Filed Jan. 8, 1954



10 FIG. 1.



11 FIG. 2.

FIG. 3.



12

FIG. 4.



13  
14

FIG. 5.



INVENTORS.

John H. Fuqua

Walter F. Sicha

Emil Veselik

By: Brown, Jackson, Boettcher & Danner

Attn:

# United States Patent Office

2,773,761

Patented Dec. 11, 1956

1

2,773,761

## FERROUS CHROME ALLOY

John H. Fuqua, Calumet City, Ill., Walter F. Jicha, Hammond, Ind., and Emil Veselik, Chicago, Ill., assignors to Calumet Steel Castings Corporation, Hammond, Ind., a corporation of Indiana

Application January 8, 1954, Serial No. 402,888

3 Claims. (Cl. 75—126)

This invention relates to iron alloys and particularly to ferrous chrome materials especially adapted for castings.

The material of our present invention is a metal alloy of the ferrous chrome class and while from an analysis of its constituents it resembles iron in some respects, likewise it approaches somewhat steel. It is our conclusion that the particular features and analysis of our substance places the same in a category somewhere between an iron and steel, considered from the standpoint of carbon content.

Basically our improved product comprises the combination of several ingredients, chief of which are carbon, chrome, molybdenum, silicon, manganese and iron combined in a designated range of proportions, as will be set forth hereinafter. Our new alloy is particularly adapted for use in castings. Generally speaking, it has been our experience that this material in its "as cast" condition, displays no unexpected properties, but that following special heat treating and quenching, outstanding hardness and resistance to wear are experienced. Further, it is interesting to note that the material displays a marked ability to work harden which suggests its adaptation for particular classes of cast articles which experience high abrasive wear. For example, present liners and paddles for pugmills require frequent replacement because of their inability to resist the extreme abrasive wear attending their operation. Our material when used in such instances has given increases in wearability as great as 400% to 500% over previous materials used for such purposes. However, since this material is not classified as a steel, it does not display particularly outstanding resistance to shock or impact as is normally experienced with a steel casting. It is therefore our finding that it is best used for liners in various types of mixers or grinding equipment and for such items as paddles, mixing arms, etc. which are not subject to more than average impact stress, but are presently short-lived from extreme wear conditions.

The main object of our invention is to provide a new and improved ferrous-chrome alloy having outstanding resistance to abrasive wear.

Another object of our invention is to provide a new and improved ferrous-chrome alloy which is capable of being work hardened and is particularly useful for increasing the life of articles used in circumstances creating high abrasive wear.

A still further object of our invention is to provide a new and improved ferrous-chrome alloy particularly suitable for castings requiring high wear resistance; as for example, for such objects as liners, paddles, mixing arms, etc. for various types of mixers or grinding equipment.

The above and further objects and features of our invention will be more fully set forth in the descriptive materials hereinafter and its properties and features will be more fully understood with reference to the accompanying micro-structure showings as set forth in the accompanying drawings.

In the drawings:

Figure 1 is a photo-micrographic showing enlarged 500 times illustrating the "as cast" structure of our alloy wherein the same contains a matrix of unresolved pearlite;

Figure 2 is a photo-micrographic showing, similar to

2

Figure 1, displaying the effects of a specified austenization treatment on the pearlitic matrix shown in the structure of Figure 1 to produce a gamma phase matrix;

Figure 3 is a photo-micrographic showing, similar to Figure 2, of our austenized alloy enlarged 100 times after a preferential etchant has been employed to illustrate the carbides of the gamma-matrix therein;

Figure 4 is a showing magnified 1000 times of a casting made from our material to illustrate the effect of abrasion on the wear surface thereof; and

Figure 5 is another enlarged showing of our alloy magnified 1800 times showing the wear resistant surface of the casting of Figure 4, and the work hardening transformations which take place therein.

Turning now to the particulars of our improved ferrous-chrome alloy we prefer that the contents thereof, other than iron, be proportioned substantially as follows:

|            |                |
|------------|----------------|
| Carbon     | 1.8% to 2.4%   |
| Chrome     | 14.0% to 17.0% |
| Molybdenum | 1.5% to 2.0%   |
| Silicon    | 1.0% maximum   |
| Manganese  | 1.25% maximum  |

The alloy of this material, cast into useful objects of the nature hereinabove indicated, produces a micro-structure similar to that illustrated in the photo-micrographic showing of Figure 1. From that figure it will be recognized that the cast material contains a matrix 10 which is indicated by the darkened areas and comprises unresolved pearlite containing complex carbides of iron, chromium and molybdenum. This pearlitic matrix is found to have an average hardness of 39.8 Rockwell Scale C. In the particular sample of Figure 1, the magnification is some 500 times normal with the etching being produced by a 2% Nital etch solution.

With regard to the structure and properties of our chrome-ferrous alloy, the same apparently displays no surpassing property or aptitude toward wear resistance in its "as cast" state. As a result we have found it necessary to heat treat the same by subjecting the "as cast" structure of Figure 1 to temperatures in the neighborhood of 2020° F. followed by an air quench. This heat treatment austenizes the pearlitic matrix thereof shown in Figure 1 and transforms the same to gamma phase (retained austenite) as illustrated particularly in Figure 2 of the drawing at 11. It is found that the hardness of the matrix after the austenization treatment is altered to an approximately 57 Rockwell C, thereby demonstrating a marked increase over its "as cast" hardness. The photo-micrographic showing of Figure 2 is an example of the austenized structure magnified 500 times and treated with a 2% Nital etch.

With regard to the gamma phase matrix of Figure 2, reference also should be had to Figure 3 of the drawings which shows the austenized structure magnified 100 times after treatment with Aqua Regia Glycerol etch to give preferential showing of the complex carbides located in the gamma matrix, as at 12. It is believed that the presence of these carbides, which have undergone a coalescence in the austenization phase to take on a generally spherical form, explains the abnormally high hardness obtained from the austenitic gamma phase matrix.

Additionally, it is found that while the material "as cast" demonstrates an average Rockwell C reading of around 40 and after austenization a hardness of approximately 60 Rockwell C, after cold working a relative hardness of 65 Rockwell C is obtained.

Such increased hardness is due in part to the presence of the multiple carbides present in the matrix coupled with the stress and strain effects experienced from cold working the surface of the material. This observation

is borne out by examination of the micro-structure of this material, which shows that the alloy contains a large percent of iron-chromium carbides of varying complexity and forms. Since these carbides are brittle and have full hardness by nature, the same are substantially unaffected by cold working.

With regard to the cold work effect, reference should now be had to Figure 4 of the drawings for a showing of the work hardened surface of a casting made of our improved alloy, magnified 1000 times and treated with an Aqua Regia Glycerol etch. It will be noted that the complex carbides 12 have not been affected by abrasion and that the depth of penetration for the abrasive effect is evidenced substantially by the darkened matrix 13. It has been established that the depth of this penetration approximates .0005 inch, as outlined by broken line 14. This shallow surface effect is somewhat surprising, but finds an understandable explanation as set forth hereinafter.

The most common cause of work hardening effect is found in distortion of the structure which results in a concentration of various complex stresses which impart increased hardness to the material. Since the hard carbides are so prevalent in our material and exist near the surface, this distortion effect is also necessarily concentrated at or near the surface, as shown. A secondary effect causing the cold work phenomena is found in the transformation of any unstable constituents which may be present. Thus, in our present material, any gamma constituent which is present in the matrix will transform under cold working stresses. However, this transformation effect which we term "phase alteration" is more or less a submicroscopic occurrence and is not readily resolved by metallographic examination. Consequently, the resultant hardness factor caused by this phenomenon may be said to be proportional to the amount of cold work to which the material is subjected. From the above it may be concluded that since the effect of the cold working is concentrated near or at the point of contact, the hardness effect is likewise necessarily restricted to a superficial depth as shown in Figure 4. It is our belief that in our particular material a triple effect of work stresses, hard carbides and transformation or phase alteration combine to furnish the extremely hard and wear resistant properties experienced.

From Figure 5, which is a showing magnified 1800 times of the cold worked surface of Figure 4 etched with Aqua Regia Glycerol, it will be seen that our above conclusions are substantiated. Particularly, it will be noted that the effect of abrasion on the wear surface appears to be present between the massive carbides 12. Further, the cold working of the several carbides which extend to the surface itself, has been transferred to the underlying and unstable gamma phase matrix 11 to produce a transformed carbide-rich, martensitic structure, as at 15.

From our above conclusions and working experience with this material, it is our opinion that its excellent wear resistant properties are due primarily to the inherent hardness afforded by the network of complex carbides and additionally by induced hardness resulting from cold working stresses and theoretical phase changes of the gamma matrix resulting from the austenitization step carried out under the specified heat treatment to produce the carbide rich martensitic matrix.

With particular regard to the ingredients specified hereinabove for our improved ferrous-chrome alloy, the following are examples of typical "heats" for this new material:

| Heat # | Carbon | Manganese | Silicon | Chrome | Molybdenum |
|--------|--------|-----------|---------|--------|------------|
| A----- | 2.25   | 1.10      | .58     | 16.5   | 1.94       |
| B----- | 2.21   | 1.00      | .44     | 16.4   | 1.88       |
| C----- | 2.08   | 1.15      | .71     | 16.6   | 1.69       |
| D----- | 2.15   | .83       | .84     | 16.9   | 1.96       |

It is worthwhile noting that the specified carbon content is substantially lower than that found in normal iron analyses and likewise it is important that the silicon and manganese content be kept low as specified to obtain the desired results. As mentioned, it has been our experience that the micro-structure of this material demonstrates a large percentage of the iron, chromium and molybdenum carbides in varied complexity after austenitization. Our examination into this material has also shown that there are increasing amounts of precipitated carbides in the gamma matrix as the austenitizing temperature is increased from about 1300° F. to the neighborhood of 2000° F. Further, while the carbides may be said to be inherently fully hardened, so that the working of the wear surface of the material affects only the matrix, it will nevertheless be noted, that such cold work effect on the matrix is somewhat superficial. However, the triple effect of stresses, a large percentage of hard carbides and the transformation of unstable gamma phase matrix combine to give the unexpected wear resistant properties of our alloy. Therefore, even though the transformation due to cold working is superficial the same is, nonetheless, very definite and beneficial.

While we have herein shown and described the make-up and components of our improved ferrous-chrome alloy, as related to a preferred range of ingredients and a certain type of austenitizing heat treatment, it will be understood and appreciated that changes, modifications and substitutions of equivalents may be employed therein without necessarily departing from the spirit and scope of our teachings. As a consequence it is not our intention that we be limited to the particular form and specifications for our alloy as presented herein except as may appear in the following claims.

We claim:

1. A ferrous-chrome alloy for castings, characterized by an ability to work harden to substantially 65 Rockwell C, after austenitization, consisting essentially of, carbon in the proportion of 1.8% to 2.4%, chromium in the proportion of 15.0% to 17.0%, molybdenum in the proportion of 1.5% to 2.0%, silicon at a maximum of 1.0%, and manganese at a maximum of 1.25%.
  2. A ferrous chrome alloy for casting purposes characterized, as cast, by a matrix of unresolved pearlite having a Rockwell C hardness of substantially 45 and containing complex carbides of iron, chromium and molybdenum, the alloy being austenitized by air quenching from substantially 2020° F. after which the same demonstrates an ability to work-harden to substantially 65 Rockwell C, comprising, 1.8% to 2.4% carbon, 15% to 17% chromium, 1.5% to 2.0% molybdenum, 1.0% silicon maximum, 1.25% manganese maximum and the balance iron.
  3. A ferrous chrome alloy for castings characterized by an ability to work-harden after austenitization, consisting essentially of:
- |                               |         |      |
|-------------------------------|---------|------|
| Carbon                        | percent | 2.21 |
| Manganese                     | do      | 1.00 |
| Silicon                       | do      | 0.44 |
| Chromium                      | do      | 16.4 |
| Molybdenum                    | do      | 1.88 |
| Iron, balance to make up 100. |         |      |

#### References Cited in the file of this patent

#### UNITED STATES PATENTS

|           |                 |               |
|-----------|-----------------|---------------|
| 2,064,155 | Fahrenwald      | Dec. 15, 1936 |
| 2,199,096 | Berglund        | Apr. 30, 1940 |
| 2,268,426 | Schlumpf et al. | Dec. 30, 1941 |
| 2,355,726 | Harder et al.   | Aug. 15, 1944 |

#### FOREIGN PATENTS

|         |               |               |
|---------|---------------|---------------|
| 315,502 | Great Britain | July 18, 1929 |
|---------|---------------|---------------|